

XR

444,842

ADDED

T 20277

UNIT

FICE.

NATHAN J. MITCHELL, OF PHILADELPHIA, PENNSYLVANIA, ASSIGNOR OF  
ONE-HALF TO NATHAN M. LEATHERS, OF SAME PLACE.

## PAINT.

SPECIFICATION forming part of Letters Patent No. 444,842, dated January 20, 1891.

Application filed October 25, 1890. Serial No. 369,364. (No specimens.)

To all whom it may concern:

Be it known that I, NATHAN J. MITCHELL, a citizen of the United States, residing at Philadelphia, in the county of Philadelphia and State of Pennsylvania, have invented a new and useful Paint, of which the following is a specification.

My invention consists in an improvement in paints, being designed for use on shingle, board, felt, tin, and iron roofs, as well as the iron work of bridges, fences, &c.

Among the objects in view are to provide a paint that on tin and iron roofs will remain pliable and not crack or scale off, and is not affected by heat or cold, where in the ordinary paints for a similar use they soon lose their efficiency by cracking and scaling off, as it is subjected to the action of the weather. On wood (shingle or board) the paint penetrates the material, causing a smooth and glossy surface, from which water runs off at once, thereby preventing decay by saturation of water and moisture. When the paint is applied in a heated condition, it expands the pores of the material and causes a complete penetration, which will last for a great number of years, thus preserving the material that much longer than without paint. The paint when applied also penetrates under the shingles at the ends exposed, which prevents moisture from drawing up under the shingle and causing decay. On paper or felt roofs the paint also penetrates the material and prevents it from cracking or decaying, besides rendering it fire-proof.

With these general and specific objects in view my paint consists of the following ingredients—namely, coal-tar, yellow ocher, or

oxide of iron, or a suitable filler, plumbago, lime, salt, and coal-oil—which are mixed together in the following proportions: Coal-tar, one gallon; yellow ocher, oxide of iron, or a suitable filler, two pounds; plumbago, one pound; lime, one and one-half pound; salt, one pound; coal-oil, one pint.

In the preparation of this paint the above-named ingredients are thoroughly mixed together and boiled for half an hour. If conditions will not admit of boiling, which renders the paint fire-proof, linseed-oil or any other suitable oil is used in lieu of the coal-tar in the same proportion.

While I use practically the proportions above named, I do not confine myself exactly to them, as they may be varied according to the condition of the material or the roof to which it is applied.

Having thus described my invention, what I claim, and desire to secure by Letters Patent, is—

1. In a paint, the combination of a suitable vehicle for paints and a filler with plumbago, lime, salt, and coal-oil, combined in substantially the proportions specified.

2. In a paint, the combination of coal-tar, yellow ocher, plumbago, lime, salt, and coal-oil, combined in substantially the proportions specified.

In testimony that I claim the foregoing as my own I have hereto affixed my signature in presence of two witnesses.

NATHAN J. MITCHELL.

Witnesses:

THOS. R. YOUNG,  
WILLIAM J. DICKSON.

3  
6  
63  
29

444842  
NO OR CLASSIF